

Sept. 27, 1949.

P. G. CHACE

2,482,898

CORROSION-RESISTING COMPOSITE METAL

Original Filed June 23, 1941



Paul G. Chace  
Inventor  
Haynes and Koenig  
Attorneys

## UNITED STATES PATENT OFFICE

2,482,898

CORROSION-RESISTING COMPOSITE  
METAL

Paul G. Chace, Attleboro Falls, Mass., assignor to  
Metals and Controls Corporation, Attleboro,  
Mass., a corporation of Massachusetts

Original application June 23, 1941, Serial No.  
399,398, now Patent No. 2,366,178, dated Janu-  
ary 2, 1945. Divided and this application No-  
vember 11, 1944, Serial No. 563,014

7 Claims. (Cl. 29—195.5)

1

This invention relates to composite metal ele-  
ments and particularly to bimetallic elements  
which are corrosion-resisting.

This application is a division of my co-pending  
application, Serial No. 399,398 filed June 23, 1941,  
Patent 2,366,178.

Among the several objects of the present in-  
vention are the provision of a composite thermo-  
stating metal which is corrosion-resisting, which  
has an improved bond, and which has a long life  
when operating in corrosion-promoting atmos-  
pheres and mediums; the provision of composite  
thermostatic metal of the class described which  
has both good hot-rolling and good cold-rolling  
properties; and the provision of composite ther-  
mostatic metal of the type indicated which is rela-  
tively simple and economical to manufacture.  
Other objects will be in part obvious and in part  
pointed out hereinafter.

The invention accordingly comprises the in-  
gredients and combinations of ingredients, the  
proportions thereof, and features of composition,  
which will be exemplified in the products here-  
inafter described, and the scope of the application  
of which will be indicated in the following claims.

In the accompanying drawing in which is illus-  
trated one of various possible embodiments of the  
invention, the single figure is a representation  
of a bimetallic element showing a strip of iron  
chromium alloy fused throughout its length to  
a similar strip of copper silicon alloy.

Many of the thermostatic elements commonly  
in use are subject to corrosion when used in the  
presence of moisture in places such as steam  
radiators, or water mixing valves, or in other in-  
stallations where corrosion-promoting fluids or  
atmospheres come in contact with the thermo-  
static metal. As a result, such elements fre-  
quently need replacing, and inasmuch as corro-  
sion tends to reduce their activity and life, such  
corrosion may set up, unknown to the user, dan-  
gerous conditions which might result in loss of  
life or injury. To avoid this corrosion of the com-  
posite metal element, it has sometimes been cus-  
tomary in the past to treat the thermostatic metal  
surface to make it less subject to corrosion, as by  
plating it with a corrosion-resisting material,  
such as cadmium, tin, zinc, lead, or chromium.  
This, however, has the disadvantage that the  
plating increases the cost materially and does not  
assure satisfactory life for the thermostatic ele-  
ment. Furthermore, such plating is not entirely  
satisfactory since an electrovoltaic potential may  
be set up which produces pitting and eating away  
of the protective metal.

It has sometimes been the practice in the past

2

to make a composite metallic element from an iron  
alloy having a high chromium content, and a  
metal alloy having a higher coefficient of expan-  
sion. The metal used for the high coefficient of  
expansion side has been one of the brasses. The  
mechanical properties of these brasses have pre-  
sented manufacturing difficulties, which in many  
instances have prevented the manufacture of an  
adequate and satisfactory composite metal. For  
example, the cold-working properties of brass are  
so different from those of the chromium iron alloy  
that it has been difficult to satisfactorily cold-  
work the metal after it has been put together to  
form a thermostatic bimetal. Moreover, it is  
highly advantageous in the manufacture of bi-  
metal to hot-roll the material down from its thick  
ingot size to an intermediate stage. The brasses  
are not adapted to this, since their hot-rolling  
temperatures differ too much from that of the  
chromium iron alloy. The manufacture of the  
brass-chrome iron bimetal has therefore been a  
relatively expensive process compared to the  
manufacture of bimetal in accordance with the  
present invention. The ingot size of the brass-  
chrome iron bimetal must be kept small because  
of the aforementioned difficulties and properties.

Where other constituents have been proposed  
for corrosion-resisting bimetals, it has been found  
relatively impossible to directly bond the metals  
together. For this reason, an intermediate solder  
layer has been used which has led to two serious  
disadvantages. First, the use of the solder layer  
decreases the corrosion-resisting property of the  
thermostatic metal due to inferior bonding, and  
second, the solder layer decreases the strength  
of the metal at elevated temperatures, since the  
solder bond is relatively weak. Also, solder-  
bonded material is difficult to hot-roll satisfac-  
torily.

By the present invention, it is possible to accom-  
plish a direct bond between the metals, and they  
may be hot-rolled or cold-rolled in the desired  
manner. Their manufacture is accordingly eco-  
nomical, and a highly corrosion-resisting thermo-  
static metal is obtained.

According to the present invention a thermo-  
static element is provided which is corrosion-  
resisting per se, particularly to air, water and  
water vapor, thus eliminating the need for sur-  
face plating. In addition, the present invention  
provides a thermostatic element made of com-  
posite thermostatic metal of the corrosion-resist-  
ing type which has a direct bond between the  
layers thereof.

The thermostatic metal of the present inven-  
tion comprises layers of metal firmly secured to-  
gether over their entire areas by a direct bond.

One of the layers, in the present invention, comprises a corrosion-resisting metal having a low coefficient of expansion. The other layer comprises a second corrosion-resisting metal having a relatively high coefficient of expansion.

For the metal having a low coefficient of expansion a high chromium content stainless iron is employed. The composition of this alloy may be as follows:

|           | Per cent  | 10 |
|-----------|-----------|----|
| Manganese | 0.2-0.6   |    |
| Carbon    | 0.01-0.2  |    |
| Chromium  | 12-20     |    |
| Silicon   | 0-1.5     |    |
| Copper    | 0-1.5     |    |
| Iron      | Remainder |    |

For the high expansion material an alloy of copper and silicon is employed. The composition of this alloy may be as follows:

|           | Per cent | 20 |
|-----------|----------|----|
| Copper    | 96-99    |    |
| Silicon   | 0.5-4    |    |
| Manganese | 0-1      |    |
| Tin       | 0-2.5    |    |

The composite thermostatic metal of which bimetal will be described as an illustrative embodiment may be formed in any of the customary manners. It is preferably formed in one of the ways described in my co-pending application, Serial No. 399,398, filed June 23, 1941, Patent 2,366,178, reference to which is hereby made.

Referring now to the drawing, the single figure illustrates a bimetallic element composed of the two alloys discussed above. Numeral 1 represents the copper silicon alloy while 3 is the iron chromium alloy.

The tensile strength and other mechanical properties of the copper silicon alloys described are sufficiently near to the same properties of the chrome-iron alloys that the two metals work well together and may be easily cold-worked. This makes the manufacture thereof more economical. As a result of obtaining a direct bond between the metals comprising the present invention, a thermostatic metal having a higher strength, greater activity, wider usable temperature range, longer life and better corrosion-resisting properties than the corrosion-resisting bimetals hitherto known, is obtained. Former metals allegedly designed to have these desirable properties have instead been relatively weak, corrode relatively easily, are more difficult to manufacture, and in general are not satisfactory.

As specific examples of alloys which may be advantageously employed in the present invention, the following examples are given. They are illustrative only:

#### Chrome-iron Alloy No. 1

|           | Per cent  |  |
|-----------|-----------|--|
| Manganese | 0.2-0.6   |  |
| Carbon    | 0.01-0.2  |  |
| Chromium  | 12-20     |  |
| Silicon   | 0-1.5     |  |
| Copper    | 0-1.5     |  |
| Iron      | Remainder |  |

#### Chrome-iron Alloy No. 2

|           | Per cent | 70 |
|-----------|----------|----|
| Manganese | 0.4      |    |
| Carbon    | 0.05     |    |
| Chromium  | 16       |    |
| Silicon   | 1        |    |
| Copper    | 1        |    |
| Iron      | Balance  |    |

#### Chrome-iron Alloy No. 3

|           | Per cent |
|-----------|----------|
| Manganese | 0.4      |
| Carbon    | 0.05     |
| Chromium  | 12-16    |
| Silicon   | 1        |
| Copper    | 1        |
| Iron      | Balance  |

#### Copper-silicon Alloy No. 1

|         | Per cent |
|---------|----------|
| Copper  | 96-98    |
| Silicon | 2-4      |

#### Copper-silicon Alloy No. 2

|         | Per cent |
|---------|----------|
| Copper  | 97       |
| Silicon | 3        |

Attention is directed to my copending applications, Serial Nos. 563,013, 563,015 and 563,016, all filed November 11, 1944.

In view of the above it will be seen that the several objects of the invention are achieved and other advantageous results attained.

As many changes could be made in the above alloys without departing from the scope of the invention, it is intended that all matter contained in the above description shall be interpreted as illustrative and not in a limiting sense.

I claim:

1. A corrosion-resisting thermostatic metal composed of an alloy having essentially the following composition:

|           | Per cent  |
|-----------|-----------|
| Manganese | 0.2-0.6   |
| Carbon    | 0.01-0.2  |
| Chromium  | 12-20     |
| Silicon   | 2-1.5     |
| Copper    | 5-15      |
| Iron      | Remainder |

and an alloy having essentially the following composition:

|         | Per cent |
|---------|----------|
| Copper  | 96-98    |
| Silicon | 2-4      |

the surfaces of said alloys being fused together at the junction.

2. A corrosion-resisting thermostatic metal composed of an iron alloy containing: manganese approximately 0.2-0.6%, carbon approximately 0.01-0.2%, chromium approximately 12-20%, silicon approximately 0.2-1.5%, copper approximately 0.1-1.5%, and the balance iron; and a copper alloy containing: silicon approximately 0.5-4%, and the balance copper; the surfaces of said alloys being fused together at the junction.

3. A corrosion-resisting thermostatic metal composed of an alloy having essentially the following composition:

|           | Per cent  |
|-----------|-----------|
| Manganese | 0.4       |
| Carbon    | 0.05      |
| Chromium  | 16        |
| Silicon   | 1         |
| Copper    | 1         |
| Iron      | Remainder |

and an alloy having essentially the following composition:

|         | Per cent |
|---------|----------|
| Copper  | 96-98    |
| Silicon | 2-4      |

the surfaces of said alloys being fused together at the junction.

4. A corrosion-resisting thermostatic metal composed of an alloy having essentially the following composition:

|           | Per cent  |    |
|-----------|-----------|----|
| Manganese | 0.4       | 5  |
| Carbon    | 0.05      |    |
| Chromium  | 12-16     |    |
| Silicon   | 1         |    |
| Copper    | 1         |    |
| Iron      | Remainder | 10 |

and an alloy having essentially the following composition:

|         | Per cent |    |
|---------|----------|----|
| Copper  | 96-98    | 15 |
| Silicon | 2-4      |    |

the surfaces of said alloys being fused together at the junction.

5. A corrosion-resisting thermostatic metal composed of an alloy having essentially the following composition:

|           | Per cent  |    |
|-----------|-----------|----|
| Manganese | 0.2-0.6   | 20 |
| Carbon    | 0.01-0.2  |    |
| Chromium  | 12-20     | 25 |
| Silicon   | .2-1.5    |    |
| Copper    | .5-1.5    |    |
| Iron      | Remainder |    |

and an alloy having essentially the following composition:

|         | Per cent |    |
|---------|----------|----|
| Copper  | 97       | 30 |
| Silicon | 3        |    |

the surfaces of said alloys being fused together at the junction.

6. A corrosion-resisting thermostatic metal composed of an alloy having essentially the following composition:

|           | Per cent  |    |
|-----------|-----------|----|
| Manganese | 0.4       | 40 |
| Carbon    | 0.05      |    |
| Chromium  | 16        |    |
| Silicon   | 1         |    |
| Copper    | 1         | 45 |
| Iron      | Remainder |    |

and an alloy having essentially the following composition:

|         | Per cent |
|---------|----------|
| Copper  | 97       |
| Silicon | 3        |

the surfaces of said alloys being fused together at the junction.

7. A corrosion-resisting thermostatic metal composed of an alloy having essentially the following composition:

|           | Per cent  |
|-----------|-----------|
| Manganese | 0.4       |
| Carbon    | 0.05      |
| Chromium  | 12-16     |
| Silicon   | 1         |
| Copper    | 1         |
| Iron      | Remainder |

and an alloy having essentially the following composition:

|         | Per cent |
|---------|----------|
| Copper  | 97       |
| Silicon | 3        |

the surfaces of said alloys being fused together at the junction.

PAUL G. CHACE.

#### REFERENCES CITED

30 The following references are of record in the file of this patent:

#### UNITED STATES PATENTS

| Number    | Name     | Date          |
|-----------|----------|---------------|
| 1,650,951 | Matthews | Nov. 29, 1927 |
| 1,948,121 | Matthews | Feb. 20, 1934 |
| 1,991,438 | Wohrman  | Feb. 19, 1935 |
| 2,075,014 | Bassett  | Mar. 30, 1937 |
| 2,087,431 | Feild    | July 20, 1937 |

#### OTHER REFERENCES

Pages 1000-1002 of The Making, Shaping, and Treating of Steel, 5th ed., 1940, pub. by Carnegie-Ill. Steel Corp., Pittsburgh, Pa.